

## UNITED STATES PATENT OFFICE

2,175,620

TREATMENT OF SHEETS, THIN BARS, AND  
THE LIKERussell R. Smith, Hillard E. Miller, and Ralph  
H. Gelder, Ashland, Ky., assignors to The  
American Rolling Mill Company, Middletown,  
Ohio, a corporation of OhioNo Drawing. Application March 10, 1937,  
Serial No. 130,216

## 1 Claim. (Cl. 148—8)

Our invention relates to a treatment for sheets, thin bars and the like, by which we prepare them for such subsequent treatment as enameling, painting, ducoing, bonderizing, nickel-plating, galvanizing, cadmium plating and alloy plating. Sheets which are ultimately to be used for any of the above named purposes must be of very high quality, in order that the various coatings will adhere well to the base metal. It is then necessary to reduce the metal to the proper thickness and to have the final sheet perfectly clean, so that it will bond with the coating which is to be applied.

Briefly, we prefer to carry out our process on sheets, strips, thin bar and the like in the following manner: Commencing with a slab, we hot roll this slab, for example, on a continuous hot strip mill or a hot sheet jobbing mill, to thin bar gauge. We then pickle the material and then reduce it to final sheet gauge either on a cold or a hot mill. If the preliminary steps of this process as above outlined have been carried on so that we now have a long strip of metal, we may proceed directly to normalize, while if we have short lengths of metal, we prefer to stitch them so as to produce a long strip. We then normalize the strip and pickle it. We then preferably pass the strip through a hydraulic spray of cold water at high pressure (for example 300 lbs. per square inch) and then through a low pressure cold water spray (for example 80 lbs. per square inch) in order to wash it. We then pass the sheets or strip through a tank containing a cyanide solution and then again wash the strip and dry it by passing it through parallel high pressure jets delivering either hot air, steam, or high pressure hot water, and then through a drying furnace which is maintained at a temperature sufficient to complete the drying of the sheet. The sheets may then pass through several loop pits and are then sheared to length.

It will be noted that in the above series of steps, we pass the sheets or strip through a tank containing a cyanide solution. The purpose of this cyanide solution is to neutralize the sheets after the pickling step. It has been usual to use a lime bath for pickling purposes, but we have found that a lime bath is not always satisfactory because it merely neutralizes the portions of free acid which remain on the sheets and does not remove the usual pickling deposit or smudge. Furthermore, since lime is but slightly soluble in water, it adheres to the sheet as free lime which later causes trouble because it promotes rust and has other detrimental effects, in the event

that the sheet is later enameled, plated, bonderized or otherwise treated.

Since the pickling bath usually contains sulphuric acid, either alone or in combination with other acids such as muriatic acid, the reaction of the acid on iron or steel will form sulphates or chlorides which are not removable with lime.

We have found that the various above mentioned deleterious results may be eliminated by a cyanide neutralizing bath. For this purpose, we prefer to use sodium cyanide, although potassium cyanide or other cyanide solutions will accomplish the same purpose. The afore-mentioned sulphates are readily soluble in a solution of sodium cyanide and they are therefore removed from the surface of the sheet and the sheet is left chemically clean.

The neutralizing bath, which contains a suitable cyanide such as sodium cyanide, is preferably held at a temperature of from 140 to 180° F. although higher or lower temperatures may be used, and is maintained at a strength of from .120 to .150 ounce of sodium cyanide per gallon of solution. The temperature of the bath will depend upon the type of drying to which the product is to be subjected, and also upon the concentration of the solution. We have found that very much weaker concentrations may be used and also that concentrations up to one or more ounces per gallon could be used. Experience has shown, however, that increased amounts of sodium cyanide do not materially improve the product. The sheets are immersed in the cyanide tank from four to five seconds, up to thirty-five or forty seconds, depending on the speed with which the strip passes through the tank. The speed with which the strip passes through the tank is a function of the preceding operations, namely normalizing and pickling.

An after treatment of cyanide neutralized sheets may comprise, for example, a temper roll through one or more passes of temper mills, which may be of the two, three or four-high variety. These passes may be made with water, with steam, with gas, or dry. The sheets may then be roller levelled. Another after treatment which we have found to be desirable involves the after treatment discussed above, followed by box annealing at temperatures from 809 to 1450° F. sheet temperature. Various gases may be introduced into the annealing box to prevent oxidation of the sheet surface.

Another after treatment which we have found desirable may include the treatments above outlined, followed by a further temper rolling on

two-, three-, or four-high mills, either wet or dry or both, and a roller leveling.

We have found that the box annealing step changes any traces of sodium cyanide which may remain on the sheet into sodium carbonate.

Where the sheets are to be subsequently galvanized, they are prepared as outlined above. Various routings may be used preceding the cyanide treatment, depending on the temper required in the galvanized product. After the cyanide treatment, the sheets are dried by one or more of the aforesaid mentioned drying media and roller leveled in preparation for the galvanizing operation. We have found that cyanide treated sheets are free from injurious sulphates and as a result the characteristics of the galvanized product are very much improved. We have noted an improved adherence of the galvanized coating and have been able to obtain a better control of the coating and an improved appearance. The galvanizing operation may, of course, be done with sheets or coils.

We may use our sodium cyanide neutralizing in the preparation of thin bar for cold reduction either in sheets or coils. For this purpose the sodium cyanide is used as a neutralized after pickling, as above outlined, and the sheets rolled from thin bar so treated, will have a better appearance due to the fact that a clean white thin

bar is used. In this product we have noted improved bonderizing characteristics, improved enamel bonding, improved plating characteristics and greater resistance to rust. The thin bar referred to above, may vary from .050 to .250 in thickness and may be up to 96 inches wide.

The above mentioned cold reduced sheet may be used with the heat treatment or it may be normalized and box annealed at various temperatures up to 1450° F. or it may be box annealed alone. In addition, various tempering processes may be included at certain stages of the operation.

It is to be understood that modifications may be made in our process without departing from the spirit of our invention and that we intend to be limited only by the appended claim.

What we claim as new and desire to secure by Letters Patent is:

A process of cyanide neutralizing pickled iron and steel sheets to be subsequently coated, in which the cyanide solution is maintained at a temperature from 140° F. to 180° F., at a concentration of from .120 to .150 ounce per gallon of solution, and in which the duration of the neutralizing step is from 4 to 40 seconds.

RUSSELL R. SMITH.

HILLARD E. MILLER.

RALPH H. GELDER.